

May 7, 1963

J. F. HASEMAN ET AL

3,088,590

WET BENEFICIATING OF PHOSPHATE ORES

Filed Sept. 2, 1960



Inventors:  
Joseph F. Haseman  
John L. Reuss  
By:  
Attorney

## 1

3,088,590

## WET BENEFICIATING OF PHOSPHATE ORES

Joseph F. Haseman, Lakeland, Fla., and John L. Reuss, Zion, Ill., assignors to International Minerals & Chemical Corporation, a corporation of New York  
Filed Sept. 2, 1960, Ser. No. 53,527  
14 Claims. (Cl. 209—12)

This invention relates to the beneficiation of phosphate ores. More particularly, the invention relates to a process for the wet concentration of unsized phosphate minerals pursuant to which a substantial portion of the phosphate values of the ore are recovered.

Wet beneficiation of phosphate ores has long been a common expedient widely practiced in the industry. Ore ground to substantial liberation of its mineral values, for example to —12 mesh, conventionally is sized by means of classifiers, screens, trommels, hydroseparation and the like to provide a —12 +35 fraction and —35 +150 or 200 mesh fraction. The coarser fraction, generally considered to be too coarse for froth flotation, is beneficiated by means of spirals, shaking tables and the like. The finer —35 mesh fraction is subjected to froth flotation.

Early practice in the concentration of phosphate ores comprising apatite or fluorapatite and a siliceous gangue entailed reagentizing the liberated finely divided ore with an anionic reagent effective selectively to coat at least a portion of the surfaces of the phosphatic particles present, followed by concentration of the reagentized ore by froth flotation to provide a phosphate concentrate as a froth product and a silica tail as a depressed or sink product. At acceptable levels of recovery, particularly from relatively low grade ores, the grade of the concentrates was objectionably low.

An alternative procedure known to the early art embraced reagentizing the liberated phosphate ore with a cationic reagent effective selectively to coat at least a portion of the surfaces of the silica particles, followed by froth flotation to produce a silica tail as a froth product and a phosphate concentrate depressed or sink product. Such a procedure likewise failed to afford a concentrate of satisfactory grade and recovery.

The phosphate industry, accordingly, resorted to a combined process pursuant to which the liberated phosphate ores were subjected to both an anionic flotation and a cationic flotation in an effort to achieve satisfactory recovery of the phosphate values.

The development which led to a first anionic flotation followed by a cationic flotation is described in detail in Crago Patent 2,293,640, and in a plurality of subsequently issued patents, including Duke—2,461,813, Duke—2,661,842, and Hunter—2,750,036. Such flotation processes reflect the recognition by the art that only the more finely divided ore, e.g., —35 mesh, is well suited for flotation.

A second line of development for the flotation of phosphate ores, wherein the phosphate ore is subjected to a first cationic flotation and then to a subsequent anionic flotation, is exemplified, *inter alia*, in Tartaron—2,222,728, Greene—2,288,237, and Hollingsworth—2,815,859. Again the processes were practiced on a rather finely divided ore, generally —20 mesh or finer.

Processes, such as the above, must rely on an arcuate sizing of the liberated ore to achieve efficient separation. In practice, however, it is extremely difficult to achieve an accurate sizing of the ore. As a threshold matter, much of the ground ore is characterized by a size of about 35 mesh. Moreover, variations in the shape and specific gravity of the particles and their tendency to blind screens further contribute to an inaccurate sizing and ultimately to a lower recovery of the phosphate values of the ore.

5

## 2

Typical screen sizings of a liberated phosphate ore are as follows:

| Mesh size | Coarse fraction, percent | Fine fraction, percent |
|-----------|--------------------------|------------------------|
| +35       | 60-40                    | 5-15                   |
| -35       | 40-60                    | 95-85                  |

10

It will be apparent such processing, requiring extensive sizing equipment, does not provide an efficient sizing of the ore.

15 It is a primary object of this invention to provide a method for the wet beneficiation of phosphate ores pursuant to which high recoveries of phosphate values are realized.

20 It is another object of this invention to provide a method for the wet beneficiation of unsized phosphate ores pursuant to which a high proportion of the phosphate values are recovered.

25 It is a further object of this invention to provide a method for the wet beneficiation of phosphate ores which does not require that the entire ground ore be subjected to a preliminary sizing.

30 In accordance with this invention, there is provided a method of beneficiating phosphate ore, which comprises:

35 (1) Subjecting unsized liberated phosphate ore to froth flotation in the presence of a cationic reagent to provide a phosphate-rich underflow and a silica containing overflow.

(2) Subjecting the underflow from (1) to froth flotation in the presence of an anionic flotation reagent to provide a phosphate-rich overflow concentrate and an underflow.

(3) Subjecting the underflow from (2) to gravity separation to provide a phosphate-rich concentrate and a silica tail.

40 This invention at the same time eliminates the preliminary sizing operation and improves the recovery of phosphate values from the ore. Accordingly, it provides a simplified process that recovers optimum quantities of the desirable constituent of the ore. Moreover, because the cationic float is accomplished first, the amount of anionic reagent required may be reduced and the acid scrub to remove anionic reagent often may be omitted.

45 From the standpoint of equipment requirements, this invention eliminates the preliminary screens or like sizing equipment and may reduce the gravity separation capacity requirement.

50 The process of this invention effectively combined froth flotation with gravity separation to provide a process which efficiently beneficiates unsized phosphate ore. In contrast to the combined cationic and anionic flotation processes referred to earlier, the process of this invention utilizes the dual ability of a flotation unit to recover a desired concentrate and to effect a sizing of the ore being processed. Predominantly silica fines are removed from the ore in the cationic flotation, and the finer phosphate particles are removed from the ore in the anionic flotation. This combined processing provides an underflow from the anionic flotation, which contains significant amounts of the coarser particles of both the phosphate values and the silica values of the ore. The underflow most effectively 55 can be processed by gravity separation. Accordingly, the process of this invention differs in principle from those processes which utilize essentially only froth flotation as exemplified, for example, by Crago or by Tartaron described above.

60 Since the process of this invention is designed to treat an unsized ore so as to yield a product stream containing

a significant proportion of the coarser particles of the ore, it will be apparent that the process of this invention also differs in principle from processes such as are exemplified by Evans—2,553,905 wherein the ore is subjected to a single flotation before gravity separation merely to eliminate a portion of one of the values.

This invention is generically applicable, without limitation, to phosphate ores amenable to wet concentration. Specific ores contemplated include Florida pebble phosphate, the various Tennessee phosphates, hard rock phosphates indigenous to the western United States, and the various foreign phosphate ores such as Moroccan phosphates.

The phosphate ore to be treated in accordance with the process of this invention is preliminarily ground employing a standard grinding apparatus to a desired mesh size, generally of at least about —10, preferably about —12, and is washed to remove slimes and provide a ground ore characterized by a mesh size of about —10 or 12, +150 or 100. Since the process of this invention efficiently processes such coarsely ground ores, the practice of this invention eliminates the need for extensive grinding to provide a very fine particle size.

The ground deslimed ore then is reagentized employing any of the cationic or positive ion agents known to the art. Such reagents include, inter alia, the higher aliphatic amines and their salts with water-soluble acids; the esters of amino alcohols with high molecular weight fatty acids and their salts with water-soluble acids; the higher alkyl-O-substituted isoureas and their salts with water-soluble acids; the higher aliphatic quaternary ammonium bases and their salts with water-soluble acids; the higher alkyl-pyridinium water-soluble acids; the higher alkyl quinolinium salts of water-soluble acids; and the like.

The reagentized ore is subjected to froth flotation employing any of the flotation equipment known to the art. The flotation is effective to remove, in the overflow, a substantial portion of the finer silica particles of the ore.

The underflow from the flotation unit, containing substantially all of the phosphate values of the ore, may, if desired or appropriate, be treated with a material such as sodium hypochlorite or the like and washed to remove the cationic reagent. While such treatment tends to improve the efficiency of the later flotation stages, it is not essential and significant recoveries can be achieved without de-reagentizing the ore after the cationic flotation.

The underflow next is subjected to froth flotation in the presence of an anionic flotation reagent to provide a phosphate overflow which contains a substantial amount of the finer phosphate particles of the ore. The underflow from the anionic flotation will contain both phosphate and silica particles and will contain a substantial proportion of the larger size particles of the original ore.

The invention generically embraces the anionic or negative ion reagents known to the art. Such reagents include, inter alia, fatty acids or fatty acids soaps, particularly mixed fatty acids or soaps thereof; fatty acids or soaps of acids derived from natural sources such as tall oil soaps and floating soap; fatty acids or soaps of acids derived from animal and vegetable fats; esters of inorganic acids with high molecular weight alcohols; and the like. Conventionally, such anionic reagents are applied in solution or in a dispersion in a carrier medium such as a hydrocarbon oil, normally kerosene or fuel oil. One widely used specific reagent combination comprises about one to about three parts tall oil, from about two to about four parts kerosene, and from about two to about four parts "Bunker C" fuel oil.

The underflow from the anionic flotation may be subjected, if it is desired or appropriate, to scrubbing with water or more desirably with a mineral acid such as sulfuric acid to remove the anionic reagent. The underflow then may be reagentized with a cationic reagent such as described above in order to increase the efficiency of the gravity separation. While the removal of the anionic

reagent tends to improve the efficiency of the gravity separation when the ore is reagentized with cationic agents, such removal is not essential.

Alternately, the underflow from the anionic flotation may be subjected to gravity separation containing only that amount of anionic reagent which is present as a result of the anionic flotation. If desired, of course, an additional amount of anionic agent can be added to the ore.

10 The underflow is subjected to a gravity separation to provide a second phosphate-rich concentrate product and a silica tail. The gravity separation may be carried out employing any of the means known to the art, including without limitation, spirals, tables, belts and the like. Spirals, for example Humphrey spirals, are found to be particularly appropriate for the gravity separation.

15 While each flotation has been described as if it were conducted in a single flotation unit, it will be apparent that a plurality of units in parallel or in series may be employed for each flotation stage. Thus, for example, the phosphate concentrate overflow from the anionic flotation can be subjected to a cleaner anionic flotation. In this event, the underflow from each unit is combined and subjected to gravity separation.

20 25 The control of flotation air rates, solids content of the slurry in the flotation unit and similar process conditions are within the skill of the routineer. Tests indicates that the cationic reagent most appropriately may be employed in amounts of at least 0.2 pound per ton and desirably in amounts of at least about 0.3 pound per ton. The 30 cationic underflow most appropriately may be conditioned with an anionic reagent in amounts of at least about 0.2 pound per ton and preferably of at least about 0.5 pound per ton. These reagents may be employed in 35 amounts up to 10 pounds per ton or more if desired. The use of large quantities of reagent, of course, tends to effect adversely the economics of the process.

25 30 The method of this invention is demonstrated by the flow sheet in the attached drawing. FIGURE 1 represents a diagrammatic flow sheet of one preferred method of this invention.

35 Referring to FIGURE 1, the deslimed unsized phosphate ore (—10 +150) from feedbin 1 is mixed with a flotation reagent composition such as a long chain aliphatic amine and delivered to flotation unit 2. The overflow 40 from flotation unit 2 will be composed primarily of silica and heavy minerals, and may either be discarded or further processed to recover heavy minerals, feldspar or the like. The underflow from flotation unit 2 is thickened, for example to a solids content of 75%, at dewatering station 3, mixed with sodium hypochlorite at 45 mixing station 4 and washed at washing station 5. The sodium hypochlorite treatment may be omitted if desired. The underflow then is conditioned with an anionic 50 flotation reagent such as tall oil and subjected to anionic flotation in flotation unit 6. The phosphate-rich overflow from flotation unit 6 may be subjected to a cleaner flotation in flotation unit 7 to provide a final phosphate overflow product. The underflows from flotation units 6 and 55 7 containing coarse phosphate and coarse silica particles are combined, dewatered at dewatering station 8, and, if desired, mixed with a mineral acid such as sulfuric acid at mixing station 9. Following a wash in washing station 10, the underflow may be conditioned with a cationic reagent. 60 65 Alternatively, stations 9 and 10 can both be omitted and the underflow subjected to gravity separation with or without added anionic reagents. The gravity concentration 11 most desirably is effected by means of spirals 70 to provide a phosphate-rich concentrate product and a silica tail.

75 The following examples are included in order more fully to demonstrate the practice of this invention. These examples are included for illustrative purposes only and are in no way intended to limit the scope of the invention.

## 5

## EXAMPLE I

Deslimed phosphate ore ( $-10 + 150$  containing about 20% +35 mesh material) was subjected to froth flotation employing 0.25 lb./ton of an amine reagent (50% aliphatic amines + 50% rosin amines) and 0.20 lb./ton NaOH.

The concentrate and tail analyzed as follows:

Table 1

|                  | Weight, gm. | Weight, percent | Assay percent |        | 10 |
|------------------|-------------|-----------------|---------------|--------|----|
|                  |             |                 | BPL           | Insol. |    |
|                  |             |                 | BPL           | Insol. |    |
| Concentrate..... | 21,570      | 52.82           | 53.97         | 27.45  |    |
| Tail.....        | 19,270      | 47.18           | 1.98          | 96.62  | 15 |

The concentrate was de-reagentized with 1.5 lbs./ton of sodium hypochlorite, washed and conditioned at 70% solids with 0.55 lb./ton of tall oil and 0.5 lb./ton NaOH for 1 minute. A rougher froth flotation followed by a cleaner froth flotation of the rougher overflow produced the following streams.

Table 2

| Stream            | Weight, gms. | Weight, percent | Assay BPL | Percent insol. | Units BPL | Units insol. |
|-------------------|--------------|-----------------|-----------|----------------|-----------|--------------|
| Cleaner conc..... | 8,272        | 48.79           | 73.71     | 2.91           | 35.96     | 1.42         |
| Rougher tail..... | 6,006        | 35.42           | 26.55     | 63.52          | 9.40      | 22.50        |
| Cleaner tail..... | 2,677        | 15.79           | 54.41     | 27.95          | 8.59      | 4.41         |

The combined tails then were subjected to spiral separation to provide a final concentrate.

## EXAMPLE II

A screen analysis of a concentrate obtained by the cationic flotation of Example I is reflected in Table 3.

Table 3

| Size               | Weight | Weight percent | Cum. weight percent | Percent BPL | Units BPL | Percent or BPL | Percent insol. |
|--------------------|--------|----------------|---------------------|-------------|-----------|----------------|----------------|
| $-10 + 14$ .....   | 7.5    | 1.5            | 1.5                 | 70.03       | 1.75      | 3.14           | 5.41           |
| $-14 + 20$ .....   | 18.0   | 3.7            | 5.2                 | 66.65       | 2.47      | 4.44           | 10.41          |
| $-20 + 28$ .....   | 33.5   | 6.9            | 12.1                | 55.07       | 3.80      | 6.82           | 25.95          |
| $-28 + 35$ .....   | 64.0   | 13.2           | 25.3                | 42.28       | 5.58      | 10.02          | 44.07          |
| $-35 + 48$ .....   | 108.0  | 22.3           | 47.6                | 46.54       | 10.38     | 18.64          | 38.11          |
| $-48 + 65$ .....   | 113.0  | 23.3           | 70.9                | 55.61       | 12.96     | 23.28          | 26.18          |
| $-65 + 100$ .....  | 114.5  | 23.7           | 94.6                | 64.35       | 15.25     | 27.39          | 14.66          |
| $-100 + 150$ ..... | 26.0   | 5.4            | 100                 | 64.57       | 3.49      | 6.27           | 12.56          |
| Total.....         | 484.5  | 100.0          |                     | 55.68       | 100       |                |                |

Table 3 demonstrates that the +35 mesh fraction, originally about 20%, constitutes about 25% of the cationic underflow. Subsequent anionic flotation is effective to increase the proportion of the +35 mesh still further.

## EXAMPLE III

A low grade Florida phosphate ore was ground to  $-10$  mesh and was washed to remove  $-150$  mesh slimes to provide an ore containing about 20% +35 mesh material. The ore then was subjected to froth flotation in the presence of 0.25 lb./ton of a cationic flotation reagent (50% aliphatic amines and 50% rosin amines), 0.50 lb./ton of kerosene and 0.25 lb./ton of NaOH. The underflow from the cationic flotation was washed with 1.5 lbs./ton of sodium hypochlorite and subjected to additional froth flotation in the presence of 0.55 lb./ton of tall oil, 0.55 lb./ton of kerosene, 1.1 lbs./ton of Bunker C fuel oil, and 0.5 lb./ton NaOH. The overflow phosphate concentrate was cleaned once by refloating without reagent. The combined underflow from the rougher and cleaner anionic flotation were washed with 10 lbs./ton of  $H_2SO_4$ . The washed underflow was then conditioned with 0.6 lb./ton of tall oil, 0.6 lb./ton of kerosene, 1.2 lbs./ton

5

## 6

Bunker C fuel oil and 0.5 lb./ton NaOH and subjected to an agglomerate tabling on a shaking table. The results of this test, based on table middlings containing 50% of the phosphate values are reflected in Table 4.

Table 4

| Product              | Weight percent | Assay, percent |             | Units BPL | Percent recovery BPL |
|----------------------|----------------|----------------|-------------|-----------|----------------------|
|                      |                | BPL            | Acid insol. |           |                      |
| Flotation conc.....  | 25.9           | 73.7           | 2.9         | 10.08     | 65.3                 |
| Table conc.....      | 13.5           | 70.2           | 7.3         | 9.47      | 31.5                 |
| Flotation tails..... | 47.2           | 2.0            | -----       | 0.94      | 3.1                  |
| Table tails.....     | 13.4           | 4.7            | -----       | 0.63      | 2.1                  |
| Total.....           | 100.0          | -----          | -----       | 30.12     | 100.0                |

The above examples demonstrate that a very high recovery of phosphate values may be achieved in accordance with the practice of this invention. Generally, the process of this invention will permit the recovery of 90% to 95% or more of the phosphate values of ore originally containing 35 to 40% phosphate values. In contrast, a standard process which initially screens comparable ore and employs gravity separation for the +35 mesh material normally recovers only 85% to 90% of the phosphate values. Moreover the practice of this invention may permit a reduction in the anionic flotation reagent requirements.

Since modifications of this invention will be apparent to one skilled in the art, it is intended that this invention be limited only by the scope of the appended claims.

We claim:

1. The method of beneficiating an unsized phosphate ore fraction which comprises:
  - (1) Subjecting an unsized liberated deslimed phosphate ore fraction containing particles of a mesh size

of from about 10 mesh to about 200 mesh to froth flotation in the presence of a cationic reagent to provide a phosphate-rich underflow and a silica containing overflow;

(2) Subjecting the underflow from (1) to froth flotation in the presence of an anionic flotation reagent to provide a phosphate-rich overflow concentrate and an underflow; and

(3) Subjecting the underflow from (2) to gravity separation to provide a phosphate-rich concentrate and a silica tail.

2. The method of claim 1 wherein the cationic reagent is aliphatic amine.

3. The method of claim 1 wherein the anionic reagent is selected from the group consisting of fatty acids and fatty acid soaps.

4. The method of beneficiating an unsized phosphate ore fraction which comprises:

(1) Subjecting an unsized liberated deslimed phosphate ore fraction containing particles of a mesh size of from about 10 mesh to about 200 mesh to froth flotation in the presence of a cationic reagent to pro-

- vide a phosphate-rich underflow and a silica containing overflow;
- (2) Subjecting the underflow from (1) to froth flotation in the presence of an anionic flotation reagent to provide a phosphate-rich overflow concentrate and an underflow;
  - (3) Subjecting the overflow from (2) to froth flotation to provide a phosphate-rich overflow concentrate and an underflow; and
  - (4) Subjecting the underflow from (2) and (3) to gravity separation to provide a phosphate-rich concentrate and a silica tail.

5. The method of claim 4 wherein the cationic reagent is aliphatic amine.

6. The method of claim 4 wherein the anionic reagent is selected from the group consisting of fatty acids and fatty acid soaps.

7. The method of claim 4 wherein the unsized ore fraction is characterized by a mesh size range of  $-12 +150$ .

8. The method of beneficiating an unsized phosphate ore fraction which comprises:

- (1) Subjecting an unsized liberated deslimed phosphate ore fraction containing particles of a mesh size of from about 10 mesh to about 200 mesh to froth flotation in the presence of a cationic reagent to provide a phosphate-rich underflow and a silica containing overflow;
- (2) Contacting the underflow from (1) with sodium hypochlorite to remove the cationic reagent;
- (3) Subjecting the treated underflow from (1) to froth flotation in the presence of an anionic flotation reagent to provide a phosphate-rich overflow concentrate and an underflow;
- (4) Subjecting the phosphate-rich overflow from (3) to froth flotation to provide a phosphate-rich overflow concentrate and an underflow;
- (5) Subjecting the underflows from (3) and (4) to treatment with a mineral acid to remove the anionic reagent, and

(6) Subjecting the treated underflows from (3) and (4) to gravity separation to provide a phosphate-rich concentrate and a silica tail.

9. The method of claim 8 wherein the cationic reagent is an aliphatic amine and the anionic reagent is selected from the group consisting of fatty acids and fatty acid soaps.

10. The method of claim 9 wherein the unsized phosphate ore fraction is characterized by a mesh size range of about  $-12 +150$ .

11. The method of claim 1 wherein said unsized liberated deslimed phosphate ore fraction contains particles of a mesh size of from about 12 mesh to about 150 mesh.

12. The method of claim 1 wherein said unsized liberated deslimed phosphate ore fraction contains particles of a mesh size of from about 14 mesh to about 150 mesh.

13. The method of claim 4 wherein said unsized liberated deslimed phosphate ore fraction contains particles of a mesh size of from about 14 mesh to about 150 mesh.

14. The method of claim 8 wherein said unsized liberated deslimed phosphate ore fraction contains particles of a mesh size of from about 14 mesh to about 150 mesh.

#### References Cited in the file of this patent

#### UNITED STATES PATENTS

|    |           |                     |                |
|----|-----------|---------------------|----------------|
| 30 | 2,222,728 | Tartaron -----      | Nov. 26, 1940  |
|    | 2,553,905 | Evans -----         | May 22, 1951   |
|    | 2,614,692 | Lawver -----        | Oct. 21, 1952  |
|    | 2,811,254 | McGarry -----       | Oct. 29, 1957  |
|    | 2,914,173 | Le Baron -----      | Nov. 24, 1959  |
| 35 | 2,922,522 | Fenske -----        | Jan. 26, 1960  |
|    | 2,952,360 | Oberg -----         | Sept. 13, 1960 |
|    | 2,970,688 | Uhlund -----        | Feb. 7, 1961   |
|    | 3,013,664 | Hollingsworth ----- | Dec. 19, 1961  |

UNITED STATES PATENT OFFICE  
CERTIFICATE OF CORRECTION

Patent No. 3,088,590

May 7, 1963

Joseph F. Haseman et al.

It is hereby certified that error appears in the above numbered patent requiring correction and that the said Letters Patent should read as corrected below.

Column 3, line 20, for "100" read -- 200 --; column 4, line 29, after "least" insert -- about --.

Signed and sealed this 10th day of December 1963.

(SEAL)

Attest:

ERNEST W. SWIDER

Attesting Officer

EDWIN L. REYNOLDS

Acting Commissioner of Patents